

## UNITED STATES PATENT OFFICE

MILTON O. SCHUR AND BENJAMIN G. HOOS, OF BERLIN, NEW HAMPSHIRE, ASSIGNEES  
TO BROWN COMPANY, OF BERLIN, NEW HAMPSHIRE, A CORPORATION OF MAINE

## PREPARATION OF NITROCELLULOSES

No Drawing. Application filed September 3, 1931. Serial No. 561,002.

This invention relates to the preparation of nitrocelluloses using cellulose fibers of various kinds and in various physical forms as the raw material. It devolves more specifically about the "drowning" treatment with water to which the freshly nitrated cellulose fiber is subjected while still wet with a large excess of the strong mixed nitrating acids carried out of the nitrating bath.

- 10 In the preparation of nitrocelluloses, the current practice is to steep cellulose fiber in suitable physical form in a bath of mixed nitrating acids containing far more acid than that which is actually consumed by the reaction upon the cellulose fiber. After the fiber has been nitrated to the desired nitrogen content, the nitrocellulose is separated from the bath of mixed nitrating acids and the acid associated therewith is rapidly diluted with 15 large quantities of water at seasonable temperatures. This step is technically known as the "drowning" operation, because the nitrocellulose is submersed completely in large quantities of diluting water. There is good 20 reason for this sort of practice, for, in order to avoid hydrolysis and accompanying loss of the nitrocellulose, the water used for removing essentially all of the mixed nitrating acids must practically instantaneously permeate the entire nitrated charge. Otherwise, 25 local over-heating may ensue, on account of the heat of dilution of the mixed nitrating acids. The large excess of water serves as a reservoir for absorbing the heat, wherefore 30 the temperature of the drowned batch of nitrocellulose is not appreciably above that of the diluting water. For example, after a batch of cotton linters has been nitrated in the usual nitrating pot and has been centrifuged or wrung free of easily removable acid, the batch is discharged from the centrifuge into an elongated porcelain column wherein 35 it meets a stream of water under sufficient pressure to break up the fibrous mass and to disseminate large volumes of water throughout the mass. The drowned nitrocellulose issuing from the bottom of the column has practically the temperature of the diluting water, by which we mean that the temperature 40 rise in the mass is at most only a few 45
- degrees. The drowned nitrocellulose is discharged into a storage tank, from which it is then pumped to the boiling or stabilizing vats, wherein it is safe to subject the highly diluted pulpy mass to boiling temperatures, 55 because of its low acidity.
- Contrary to such prior art practice, we have discovered that it is advantageous to drown freshly nitrated cellulose associated with the strong mixed nitrating acids, not removed by draining or centrifuging, to drowning with warm water at temperatures appreciably above seasonable temperatures, but below about 45° C., as a maximum. By this sort of practice, we have found that improved 60 results are secured, principally in the clarity of the nitrocellulose solutions, when the nitrocellulose is put through the usual subsequent operations and is dissolved in the customary nitrocellulose solvents. The surprising thing 65 is that no material loss in nitrocellulose is encountered so long as we avoid overstepping a temperature of about 45° C. in the diluting or drowning water, but the loss in yield becomes increasingly more serious as the temperature is raised above 45° C.,—so much so, 70 that at about 55° C. or higher, the yield may drop 10% or 20%, or even more. In other words, the yield of nitrocellulose stays practically constant up to about 45° C., where- 75 above there is such a sharp drop in the yield that temperatures in the neighborhood of 45° C. represent a critical zone which should not be overstepped.
- While not limited thereto, our discovery is 80 of vital significance in connection with the nitration of refined wood pulps which, from the standpoint of purity, alpha cellulose content, and other characteristics, should normally yield nitrocelluloses of a quality comparable to those realized from cotton linters. 85 In the case of the best refined wood pulps, however, as is also true with cotton linters, for one reason or another, the solutions of the nitrocelluloses may have a turbidity or haziness which, of course, militates against their 90 most satisfactory use in the manufacture of many nitrocellulose ultimates, like lacquers or films. By drowning nitrocelluloses prepared from refined wood pulps in accordance 95 100

with the present invention, we are enabled to improve greatly the clarity and sparkle of the nitrocellulose solutions. Unless our invention is practised, one may not consistently secure nitrocellulose solutions of the best clarity and sparkle. Thus when the customary drowning procedure is followed, one may not run into the trouble of haziness in the nitrocellulose solution with several successive batches, but, sooner or later, one batch may be appreciably off grade when it is put into solution. This may be attributed to variations in the characteristics of the cellulose fiber, in acid composition, and in temperature, time, and other factors of nitration. While we cannot with precision account for the improved results which we secure, nevertheless our picture is that haziness in the nitrocellulose solution is frequently caused by the presence in the nitrocellulose of nitrates of low solubility in the nitrocellulose solvents. These undesirable nitrates, which may be present in only traces, are evidently hydrolyzed and removed under the conditions of acidity and temperature prevailing during the diffusion of the warm diluting or drowning water into the mass of nitrocellulose. On the other hand, the primary nitrocellulose product, which is completely soluble in the nitrocellulose solvents, is evidently unaffected under the conditions prevailing during the drowning in warm water, provided that a temperature of about 45° C. is not exceeded.

Using comparatively thick sheets of refined wood pulp, known as "drier sheets", the procedure may be about as follows. The sheets of wood pulp may be conditioned for nitration in such a way as to yield nitrocelluloses of  $\frac{1}{2}$ -second or lower solution viscosity. The conditioning treatment may, for example, comprise two steps, viz., the step of mercerization with caustic soda solutions of 18% or greater strength at about room temperature, followed by the step of hydrolysis with suitable acid, preferably dilute mineral acids, such as hydrochloric, sulphuric, or the like. Each of these major steps is followed by a washing operation in order to avoid interference with the succeeding step. The mercerized and hydrolyzed sheets are dried, and may then be steeped for about two hours at about 30° C. in a mixed nitrating acid, whose composition may, for example, be 17.0% water, 33.2% nitric acid, and 49.8% sulphuric acid. The nitrating acid may then be drained from the sheets and be replaced by another mixed nitrating acid containing 18.7% water, 20.5% nitric acid and 60.8% sulphuric acid, in which the sheets may be allowed to remain for about two hours at 30° C. The second acid may be drained from the nitrated sheets and the batch of acid-wet nitrocellulose then drowned in a large volume of water at say about 35° C. Excellent results have been obtained with a ratio of drowning water to

nitrocellulose of say, about 35 to 1, by weight, as this ensures a temperature throughout the drowned sheets safely below 45° C. The drowning water is drained from the sheets and is replaced by fresh water, in which the sheets may be boiled, as through the direct addition of live steam, in order to effect the usual stabilization. The two-step nitrating operation hereinbefore given is one which has been found to be eminently suitable for the nitration of thick sheets of refined wood pulp, as more fully disclosed in application Serial No. 451,995, filed May 13, 1930 by Milton O. Schur. One may, however, use other suitable nitrating procedures, and then follow them up with a drowning procedure with warm water in accordance with our invention. So, too, one may nitrate refined wood pulp in other forms, e. g., in bulk or shredded condition, and then subject the drained or centrifuged nitrocellulose to our novel drowning step. In such latter instances, the drowning may be effected by playing a stream of the warm water under suitable pressure onto the nitrated material so as to avoid local over-heating beyond that at which we secure our optimum results.

We claim:

1. In the preparation of nitrocelluloses, that step which comprises drowning the freshly nitrated cellulose associated with the strong mixed nitrating acids in a large volume of warm water but at a temperature not in excess of about 45° C.
2. In the preparation of nitrocelluloses from sheets of wood pulp, those steps which comprise steeping such sheets in the mixed nitrating acids, draining the acids from the sheets, and drowning the acid-wet sheets in a sufficiently large volume of warm water but at a temperature not in excess of about 45° C. to ensure practically the same temperature throughout the drowned sheets.

In testimony whereof we have affixed our signatures.

MILTON O. SCHUR.  
BENJAMIN G. HOOS.

115

120

125

130